

1,252,654.

A. G. BETTS.  
ELECTRODEPOSITION OF METALS,  
APPLICATION FILED MAY 15, 1916.

Patented Jan. 8, 1918.



Anson G. Betts  
Inventor

By his Attorneys  
Rev. Page, Cooper & Haygood

# UNITED STATES PATENT OFFICE.

ANSON G. BETTS, OF ASHEVILLE, NORTH CAROLINA.

## ELECTRODEPOSITION OF METALS.

1,252,654.

Specification of Letters Patent. Patented Jan. 8, 1918.

Application filed May 15, 1916. Serial No. 97,544.

*To all whom it may concern:*

Be it known that I, ANSON G. BETTS, a citizen of the United States, residing at Asheville, in the county of Buncombe and State of North Carolina, have invented certain new and useful Improvements in Electrodeposition of Metals, of which the following is a full, clear, and exact description.

10 This invention relates to the electrolytic recovery of metals from solutions of salts thereof, particularly zinc from acid sulfate solutions. In the electrolytic method of zinc recovery the zinc sulfate is electrolyzed with 15 suitable anodes and cathodes, with deposit of metallic zinc on the cathodes, thus liberating sulfuric acid and making the electrolyte more acid until it is finally removed from the electrolytic cell as a solution of 20 sulfuric acid containing only a little zinc sulfate.

It is well known that the amount of zinc deposited for a given consumption of current is always considerably less than the 25 amount that would be expected from theoretical considerations. In short, the efficiency of the process is undesirably low, and hence the cost undesirably high. It is accordingly the object of my present invention to provide an electrolytic process by 30 which the amount of zinc deposited with given current consumption will be increased. Another object is to diminish the amount of hydrogen liberated along with the zinc at 35 the cathode. These objects I attain by the simple expedient of giving the inner surface of the electrolytic tank, in contact with the solution, (which surface is usually metallic lead), an electric potential of its own, 40 relative to the solution, so that some current will flow from the solution to the tank as well as to the cathode. This has the effect of increasing the efficiency of the cell, that is, it permits the use of less current for a 45 given amount of zinc deposited, or, conversely, permits more zinc to be deposited with the same amount of current.

It is my present belief that the above-mentioned potential (which for convenience 50 can be referred to as the "tank potential") accomplishes the result described by (1) opposing the formation of a lead salt, more or less soluble in the zinc solution, by the acid of the zinc solution attacking the lead sur-

face of the tank, which salt, when present in 55 the solution, exerts an unfavorable effect, probably catalytic, upon the deposition of the zinc; (2) diminishing the amount of hydrogen liberated at the cathode along with the zinc, which hydrogen tends to cling to 60 the cathode and thereby increase the resistance of the cell, causing some of the current to be wasted in heating effects; and (3) hindering re-dissolving of zinc from the cathode by the free acid of the solution, that is, 65 hindering re-formation of the zinc salt by attack of the free acid upon the metallic zinc deposited on the cathode.

In the accompanying drawing I have shown diagrammatically a simple electrolytic cell for practising my method in the preferred manner. In the cell illustrated, 1 is the tank, which may be made of wood, 2 is the lead lining, and 3 designates the electrolyte, preferably an acid zinc sulfate solution. The anode and cathode are designated A and C respectively, and may be of any suitable material, for example aluminum. The cathode is electrically connected to the lead lining by wire 4. This gives the lead 70 surface a negative potential with respect to the anode or positive electrode A, with the result that current flows to the lead and thence to the negative pole as well as direct to the latter. This has the effect, in general, 75 of opposing the formation of a lead salt, which effect may possibly be explained on the theory that as fast as the lead salt is formed it is reduced by electrolytic action and the lead re-deposited on the lead surface. It also tends to deposit zinc on the lead surface, and if enough current were allowed to flow to the lead the amount of zinc 80 there deposited would be considerable. I 85 therefore prefer to include a suitable resistance R in the connection, of such value that sufficient current can flow to prevent formation of lead salt. The current may even be large enough to deposit a small 90 amount of zinc on the lead surface, but such deposit can easily be removed from time to time by means of sulfuric acid solution.

It is to be understood that the invention is not limited to the specific details herein described but can be practised in other ways 105 without departure from its spirit. Nor is the invention limited to zinc recovery, but is in general applicable to other metals that

are more soluble in the acid electrolyte used than is the metal (for example lead) used for the inner surface of the tank.

I claim:

- 5 1. The method of electrodepositing metals of greater solubility in the acid of the salt contained in the electrolyte than lead, comprising the step of electrolyzing a solution of a salt of the metal with suitable anode and cathode in a vessel having an inner surface of lead, while passing current to the lead inner surface.
- 10 2. The method of electrodepositing metals of greater solubility in the acid of the salt contained in the electrolyte than lead, comprising the step of electrolyzing a solution of a salt of the metal with suitable anode and cathode in a vessel having an inner surface of lead, while passing current from the anode to the said lead inner surface of the vessel.
- 15 3. The method of electrodepositing metal in a vessel having a lead inner surface, comprising electrolyzing in such vessel a solu-

tion of a salt of the metal while maintaining at the said lead surface a negative potential high enough to substantially prevent the formation of a lead salt thereat.

4. The method of electrodepositing zinc from its sulfate solutions, comprising electrolyzing the solution with suitable anode and cathode in a vessel having a lead inner surface, while passing current from the electrolyte to the said lead inner surface.

5. An apparatus for electrodeposition comprising a lead lined receptacle, an anode and a cathode therein, each spaced from said receptacle, a positive terminal connected to said anode and a negative terminal connected to said cathode; and an independent connection between the lead lining of said receptacle and the said negative terminal, said independent connection offering a relatively high resistance to the flow of the electric current.

In testimony whereof I hereunto affix my signature.

ANSON G. BETTS.